

# UNITED STATES PATENT OFFICE.

FRANK C. MATHERS, OF BLOOMINGTON, INDIANA.

## PROCESS FOR ELECTROLYTIC DEPOSITION OF METALS.

931,944.

Specification of Letters Patent. Patented Aug. 24, 1909.

No Drawing.

Application filed April 21, 1909. Serial No. 491,349.

To all whom it may concern:

Be it known that I, FRANK C. MATHERS, a citizen of the United States, residing at Bloomington, in the county of Monroe and 5 State of Indiana, have invented a new and useful Process for the Electrolytic Deposition of Metals, of which the following is a specification.

My invention relates to the electrolysis of 10 a solution containing a salt or salts of perchloric acid, or perchloric acid, or a mixture of perchloric acid and a salt or salts of perchloric acid with anodes of the metal or alloy that is to be plated or refined or 15 changed to an insoluble salt, or with an insoluble anode like platinum in which case the metal that is deposited upon the cathode comes from the bath which may be brought back to the proper strength in any suitable 20 manner. To form insoluble salts of the metals or alloys, the metal or alloy whose insoluble salt is to be formed is used as anode material in an electrolyte containing a salt or salts of perchloric acid or perchloric acid 25 or a mixture of perchloric acid and a salt or salts of perchloric acid. Upon electrolysis the anode material dissolves and the insoluble salt may be prepared by precipitating this soluble perchlorate thus formed with a 30 suitable reagent.

It is very desirable that a plating or refining bath should be made from salts and acids that are very soluble in water, that are stable, that is are neither oxidized nor reduced by electrolysis and are unchanged by 35 the air etc., that give good deposits upon the cathode and that give good efficiencies of corrosion at the anode and of deposition upon the cathode. Perchloric acid ( $\text{HClO}_4$ ) and its 40 salts ( $\text{RClO}_4$ ) fulfil these demands in a satisfactory manner. Perchlorates of the heavy metals are very soluble in water so that solutions may be prepared of almost any desired strength up to one part of salt in one part 45 of water in many cases which is much beyond any concentration that is ever used in commercial plating or refining by electrolysis. The acid radical of perchloric acid and of perchlorates is very stable,—it is not 50 reduced even by a zinc-copper couple neither is it oxidized under any conditions. It is only decomposed when ignited or fused, a treatment to which it need not be subjected in the process described in this specification. 55 The current efficiency at both electrodes is almost theoretical. The deposits upon the

cathode are smooth, dense and coherent. To obtain these good results, it is understood that the process must be carried out by one who is skilled in electroplating and electro-refining and who understands how to use the knowledge that is commonly practiced in these arts. For example: The solution should be circulated or stirred to prevent undue changes in concentration. The solution should be of the proper concentration and should contain the proper amount of free acid. I prefer a bath containing from 5 to 10 per cent. of metallic perchlorate and from 2 to 5 per cent. of free perchloric acid, 60 with such metals as copper, lead, silver, etc. which are easily deposited while with zinc, cadmium, etc. a lower concentration of acid should be used. If an adherent protective deposit is desired upon the cathode, the 65 cathode should be clean and free from grease. If it is desired to strip the deposited metal from the cathode, a greased cathode should be employed. The addition of small quantities of certain substances greatly improves the character of the deposit in regard to smoothness, brightness, and denseness. The beneficial effects of these substances have been long known and are described in many books and original articles upon the 70 subject. Among the substances that have been suggested as additions to the bath are:—arsenious acid, stannous chlorid, (Watt *Electrometallurgy*, 1895, page 46) carbon disulfid, collodion, iodin and gutta-percha in chloroform, etc. M'Millen, *A Treatise on Electrometallurgy* 1890, page 9). Experiments in connection with this work have shown that tannin is also an excellent addition substance. I prefer to use from 0.1 to 0.4 75 per cent. of these substances. The current density must be regulated depending upon the concentration of the solution, the amount of free acid that is present, the temperature, the amount of stirring, the nature of the metal that is to be plated or refined, etc. I prefer a density of from 20 to 30 amperes per square foot with solutions containing about 80 10 per cent. of metallic perchlorate and 5 per cent. of free perchloric acid. 85

The process described in this specification may be carried out with any suitable form of apparatus.

What I claim as new and desire to secure by Letters Patent, is:

1. That improvement in the art of electro-depositing metals which consists in subject-

ing the metal or an alloy of the metal as anode to an electric current in a solution containing a salt of perchloric acid and in electrodepositing the metal upon the cathode 5 substantially as described.

2. That improvement in the art of electrodepositing metals which consists in subjecting the metal or an alloy of the metal as anode to an electric current in a solution 10 containing salts of perchloric acid and in electrodepositing the metal upon the cathode substantially as described.

3. That improvement in the art of electrodepositing metals which consists in subjecting the metal or an alloy of the metal as anode to an electric current in a solution containing a salt of perchloric acid and of free perchloric acid and in electrodepositing the metal upon the cathode substantially as de- 20 scribed.

4. That improvement in the art of electrodepositing metals which consists in subjecting the metal or an alloy of the metal as anode to an electric current in a solution con- 25 taining salts of perchloric acid and of free perchloric acid and in electrodepositing the metal upon the cathode substantially as de- scribed.

5. That improvement in the art of electro-

depositing metals which consists in subject- 30 ing to an electric current a solution containing a salt of perchloric acid and in electrodepositing the metal contained in said salt upon the cathode substantially as described.

6. That improvement in the art of electrodepositing metals which consists in subjecting to an electric current a solution containing salts of perchloric acid and in electrodepositing the metal contained in said salt upon the cathode substantially as described. 35

7. That improvement in the art of electrodepositing metals which consists in subjecting to an electric current a solution containing a salt of perchloric acid and of free perchloric acid and in electrodepositing the 40 metal contained in said salt upon the cathode substantially as described.

8. That improvement in the art of electrodepositing metals which consists in subjecting to an electric current a solution containing salts of perchloric acid and of free perchloric acid and in electrodepositing the 45 metal contained in said salt upon the cathode substantially as described.

FRANK C. MATHERS.

Witnesses:

THOMAS J. SARE,  
ROBERT E. LYONS.